

## UNITED STATES PATENT OFFICE

2,664,355

## Ti-Mn-Fe ALLOYS

Charles M. Craighead, Columbus, Ohio, assignor, by mesne assignments, to The Battelle Development Corporation, Columbus, Ohio, a corporation of Delaware

No Drawing. Application October 6, 1950,  
Serial No. 188,892

## 2 Claims. (Cl. 75—177)

**1** This invention relates to titanium-base alloys and, in particular, to alloys of titanium containing manganese and iron, and is a continuation-in-part of co-pending application, Serial No. 36,434, filed July 1, 1948, now abandoned. Heretofore, titanium-base alloys have been little known due in part to previous scarcity of pure titanium metal and in part to the prior art teaching and belief that titanium-base alloys were not possessed of properties such as are required of structural materials or materials for other allied uses. It has now been discovered that certain titanium-base alloys possess good strength and hardness properties together with sufficient ductility to render them useful and 15 advantageous for numerous and varied uses.

It is, therefore, an object of this invention to provide new and useful titanium-base alloys.

It is a further object of this invention to provide titanium-base alloys having good mechanical properties. 20

Yet another object of this invention is to provide new titanium-base alloys containing manganese and iron.

Other objects and advantages of this invention will be apparent in view of the following 25 detailed description thereof.

In general, this invention relates to titanium-base alloys containing from about 1.0% to 5.0% manganese and from about 1.0% to about 2.0% iron. 30

Properties of alloys of the present invention have been determined and are reported in Table I below. The mechanical properties listed in Table I were measured using specimens prepared from alloys in the as-hot-rolled (at 1450° F.) condition. Properties of specimens similarly prepared from the unalloyed titanium are included for purposes of comparison.

TABLE I  
Mechanical properties of Ti-Mn-Fe alloys

| Composition <sup>1</sup> |     | Tensile strength, p. s. i. | Elongation percent in 1-inch | V. H. N. |
|--------------------------|-----|----------------------------|------------------------------|----------|
| Mn                       | Fe  |                            |                              |          |
| (2)                      | (2) | 87,500                     | 21.5                         | 205      |
| 1.75                     | 1.0 | 120,800                    | 12.0                         | 271      |
| 2.5                      | 1.0 | 170,000                    | 8.5                          | 260      |
| 3.5                      | 1.0 | 141,200                    | 10.0                         | 295      |
| 5.0                      | 1.0 | 144,300                    | 2.0                          | 315      |
| (2)                      | (2) | 87,500                     | 21.5                         | 205      |
| 1.75                     | 2.0 | 136,500                    | 8.5                          | 291      |
| 2.5                      | 2.0 | 152,000                    | 7.5                          | 336      |
| 3.5                      | 2.0 | 175,000                    | 5.5                          | 373      |
| 5.0                      | 2.0 | 180,000                    | 2.0                          | 352      |

<sup>1</sup> Balance titanium.

<sup>2</sup> Unalloyed.

**2** It has also been observed and determined that the alloys of the present invention respond to heat treatment. This has been demonstrated by observing increases in hardness which occur when the alloys are heated in air for one-half hour at temperatures at or above the rolling temperature (1450° F.) followed by a quenching in cold water. Table II below tabulates these values illustrating how the present alloys do respond to this heat treatment.

TABLE II  
Heat treating data for Ti-Mn-Fe alloys

| Composition <sup>1</sup> |     | Vickers hardness after heat treatment at— |           |           |           |           |           |
|--------------------------|-----|-------------------------------------------|-----------|-----------|-----------|-----------|-----------|
| Mn                       | Fe  | 1,450° F.                                 | 1,550° F. | 1,600° F. | 1,650° F. | 1,700° F. | 1,750° F. |
| (2)                      | (2) | 164                                       | 167       | 179       | 187       | 205       | 202       |
| 1.75                     | 1.0 | 257                                       | 344       | 327       | 401       | 429       | 437       |
| 2.5                      | 1.0 | 332                                       | 413       | 399       | 400       | 394       | 438       |
| 3.5                      | 1.0 | 411                                       | 424       | 432       | 416       | 405       | 429       |
| 5.0                      | 1.0 | 383                                       | 385       | 413       | 433       | 446       | 446       |
| 1.75                     | 2.0 | 387                                       | 502       | 451       | 481       | 473       | 499       |
| 2.5                      | 2.0 | 376                                       | 468       | 427       | 488       | 472       | 483       |
| 3.5                      | 2.0 | 390                                       | 426       | 459       | 455       | 437       | 421       |
| 5.0                      | 2.0 | 323                                       | 427       | 359       | 366       | 373       | 380       |

<sup>1</sup> Balance titanium.

<sup>2</sup> Unalloyed.

From Table II above, it will be apparent that the present alloys respond to heat-treatment as evidenced by increasing hardness after treatment. From Table I, it will be further evident that these alloys possess desirable tensile properties and good hardness, together with adequate ductility to permit working. It is believed that these alloys will also prove useful in applications requiring corrosion-resistant properties and good high-temperature characteristics. New and useful alloys of titanium having been disclosed, it is desired to claim the invention set forth in the appended claims.

What is claimed is:

**45** 1. An alloy consisting essentially of from 1.0% to 5.0% manganese, from 1.0% to 2.0% iron, and the balance titanium, characterized by a tensile strength of at least about 25% in excess of the tensile strength of unalloyed titanium, measured in the as-hot-rolled (at 1450° F.) condition.

**50** 2. An alloy consisting of from about 1.0% to about 5.0% manganese, from about 1.0% to about 2.0% iron, and the balance titanium.

CHARLES M. CRAIGHEAD.

**55** 55 References Cited in the file of this patent  
"Journal of Metals," March 1950, page 526.